

PATENTED DEC. 15, 1903.

No. 746,970.

J. W. MACDONALD.

SMELTING ORES.

APPLICATION FILED MAR. 30, 1903.

NO MODEL.



Witnesses:

H. W. W. Guffey  
S. A. Cochran

Inventor

J. W. Macdonald

## UNITED STATES PATENT OFFICE.

JOHN W. MACDONALD, OF PITTSBURG, PENNSYLVANIA, ASSIGNOR  
TO UNITED STATES SULPHIDE SMELTING FURNACE COMPANY,  
OF TOLEDO, OHIO.

## SMELTING ORES.

SPECIFICATION forming part of Letters Patent No. 746,970, dated December 15, 1903.

Application filed March 30, 1903. Serial No. 150,258. (No specimens.)

*To all whom it may concern:*

Be it known that I, JOHN W. MACDONALD, of Pittsburg, in the county of Allegheny and State of Pennsylvania, have invented new and useful Improvements in Processes of Smelting Ores; and I do hereby declare the following to be a full, clear, and exact description of said invention, reference being had to the accompanying drawings, and to the figures of reference marked thereon, which form a part of this specification.

My improvements relate more particularly to the smelting of sulfid ores carrying copper, gold, and silver, and consist in a method where-  
15 in unroasted ore is charged directly into a fusing zone of heat within a furnace and is fused down with the aid of a highly-heated air-blast and the gases given off by the ore, together with a small percentage of carbona-  
20 ceous fuel or without extraneous fuel, accord-  
ing as the ore treated be high or low in de-  
sired gaseous qualities.

I am familiar with the invaluable experimental work of Hollway in the field to which  
25 the improvement herein described particu-  
larly appertains as well as with the apparatus  
and methods of others of later date used in  
attempts to obtain practical results based  
largely upon the data secured by Hollway.  
30 The failure heretofore to develop such a  
method of smelting sulfid ores into a com-  
mercially-successful practice would seem to be  
not because of the want of knowledge of the  
metallurgy involved, but rather because of the  
35 failure to employ such mechanical methods  
as would utilize to the very fullest degree the  
well-known valuable forces to be found in  
ores of this class, a conclusion supported by  
operations now being successfully conducted  
40 on a commercial scale wherein is being prac-  
ticed my method herein described.

It is well known to those familiar with the  
art of smelting sulfid ores that a large part  
of the ordinary smelting-furnace is utilized  
45 in operations preliminary to actually fusing  
down the ore charge and that a large part of  
the cost of smelting the ore as ordinarily con-  
ducted enters into that of roasting or calcin-  
ing it. As the preliminary roasting or cal-  
50 cining of the ore is not required in operations

under this method, no burden of ore, as gen-  
erally understood, is carried in the furnace  
and none is desired, because to permit the  
presence of a body of ore above the fusing  
zone of flame would be to desulfurize the ore, 55  
and thus destroy a valuable element sought  
to be utilized in the practice of this method,  
and, further, as it is desired to get the full  
benefit of all the heat in the furnace above  
the fusing zone for the purpose of heating the 60  
air supplied to the furnace any obstruction  
above that point, such as would be a burden  
of ore, would tend to cool the escaping gases  
and render them inefficient in heating the air-  
blast. Therefore a furnace with a hearth of 65  
fifty inches need not be over sixty inches high  
above the hearth and is preferably built cy-  
lindrical in form, and in the accompanying  
drawing such a furnace is shown not in full  
detail, but sufficiently so to illustrate this 70  
method. A heating-chamber of the design  
shown in United States Patent No. 720,257  
is erected adjacent the furnace for heating  
the air-blast and is brought to a proper heat  
preliminary to charging the furnace with ore. 75

To put my method into operation, the fur-  
nace is preliminarily charged with a mixture  
of unroasted ore and carbonaceous fuel suffi-  
cient only in quantity to form a conical body 1  
and just covering the furnace-hearth, and as 80  
this charge is brought to glowing heat the  
sulfids therein will begin to give off gases,  
the flow of which will be accelerated under  
the influence of the blast, which may now be  
turned on.

As the practice of this method makes nec-  
essary the use of a large volume of air, the  
twyers 2 are unusually large and greater in  
number than would ordinarily be required  
for a furnace of this area of hearth. These 90  
twyers are of such inclination and proximity  
to the furnace-hearth that the heated air  
forced through them under the influence of  
the blast impinges upon the conical body of  
ore and carbonaceous fuel at many points 95  
about its base, which ore soon becomes highly  
incandescent with resulting copious flow of  
gases as well from its ore as from its car-  
bonaceous fuel, and these gases, coming in  
contact with the large volume of heated oxy- 100

gen entering the furnace with the blast at many points near its hearth, unite therewith to form a body of flame, which completely envelops the conical-formed body upon the 5 furnace-hearth.

The successful operation of this method 10 contemplates the air supplied the furnace reaching the twyers at a temperature approximately 600° Fahrenheit, and because of this 15 high heat the oxygen yielded up by the blast as it enters the furnace unites so rapidly with the gases coming off the incandescent ore that the several zones of resulting flame form so close to the points where the blast enters 20 the furnace that the fusing zone of the flame has its base very close to the furnace-hearth, and as the blast enters at many points around the hearth the base of the fusing zone circles that of the incandescent conical body of ore 25 and, rising about said ore-body, forms a mantle 3 of intense heat, which wholly envelops it, and if the conditions herein described, and consequent upon which this zone of intense heat has been created, are maintained the 30 said fusing zone of flame will always assume and retain the configuration of the conical body of ore upon the furnace-hearth and within which zone of heat the operation of fusing down the ore to a liquid mass will take 35 place.

While Hollway's work demonstrated that with proper methods it would be possible to fuse unroasted sulfid ores without extraneous fuel, his work very clearly demonstrated the 40 impracticability of accomplishing this result in any manner in which the ore would be exposed to rapid oxidation before fusion, which conclusion has been confirmed by later experimenters, notably when it has been attempted to carry on such fusion in furnaces in which reduction, fusion, and conversion take place, not designedly so, but necessarily so, to a more or less extent.

As this method is designed to operate only 45 upon ores of a character suited to it and performs but one step in recovering the metal from such ore—namely, fusing down the ore to a liquid mass from which the metal compounds may be readily recovered by gravity for subsequent further treatment, and to bring about this fusion without material preliminary oxidation of the ore operated upon, and while this ore is in a furnace filled largely 50 with an oxidizing-flame—reasonable care is required to be exercised to charge the furnace with small quantities of ore at short intervals, to the end that the ore-body upon the 55 furnace-hearth may retain the conical form herein described and that the flow of air entering the furnace be so regulated as that the fusing zone of flame will always be of such volume as to completely envelop the ore-body.

As is well known in creating a fusing zone 60 of flame in the manner here described, an oxidizing-flame is also produced which will form the enveloping-mantle 4 of the fusing

zone; but as the movement of this oxidizing zone of flame is in a direction away from the ore upon the furnace-hearth the ore will, so 70 long as such a zone is maintained above the ore, be free from attack by the oxidizing-flame, and thus the operation of fusion will go on without material oxidation that would result in elimination of the non-volatile sulfur, and if an ore be sufficiently high in sulfids and be otherwise suitable to be handled by this method operations may be continued indefinitely without the use of extraneous fuel by successively charging unroasted ore 75 directly into the fusing zone of flame at short intervals and in such quantities as may be required to maintain the form and proportions of the ore-body upon the furnace-hearth as the ore charge is fused down to a liquid 80 mass, and by supplying such a volume of heated oxygen to the furnace as that when the same combines with the gases given off by said ore charge such a flame of heat will be created as will form a fusing zone of sufficient 85 volume to wholly envelop the ore to be fused down.

Having now described my invention, I claim—

1. The process of smelting sulfid ores, which 90 consists in placing an initial charge of the raw sulfid ore on a hearth, the inclined sides comprising the upper surface of the charge being exposed, heating the charge to a temperature sufficient to enable a portion of the 95 sulfur therein to combine with oxygen, forcing air upon the exposed inclined sides of the surface of the charge, thereby effecting combustion of a portion of the sulfur and enveloping the charge in a mantle of flame 100 and fusing the outer portions of the charge, and feeding successive portions of raw ore upon the surface of the charge to maintain the charge constantly in the form having inclined sides to receive the air upon its surface, and drawing off the molten product, as 105 required.

2. The process of smelting sulfid ores, which 110 consists in placing an initial charge of the raw sulfid ore on a hearth, the inclined sides 115 comprising the upper surface of the charge being exposed, heating the charge to a temperature sufficient to enable a portion of the sulfur therein to combine with oxygen, causing several streams of air to impinge upon 120 the upper surface of the base of the charge and thence rise along its exposed surface, thereby effecting combustion of a portion of the sulfur and enveloping the charge in a mantle of flame and fusing the outer portions of the charge, and feeding successive 125 portions of raw ore upon the surface of the charge and drawing off the molten product, as required.

3. The process of smelting sulfid ores which 130 consists in placing a conical heap of the raw sulfid ore on a hearth, with its inclined sides exposed, heating the heap to a temperature sufficient to enable a portion of the sulfur

therein to combine with oxygen, forcing air upon the exposed sides of the heap, thereby effecting combustion of a portion of the sulfur and enveloping the heap in a mantle of flame and fusing the outer portion of the heap, and feeding successive portions of raw ore upon the surface of the heap and drawing off the molten product, as required.

4. The process of smelting sulfid ores, which 10 consists in placing a conical heap of the raw sulfid ore on a hearth, with its inclined sides exposed, heating the heap to a temperature sufficient to enable a portion of the sulfur therein to combine with oxygen, causing several streams of hot air to impinge upon the

base of the heap and thence rise along its exposed surface, thereby effecting combustion of a portion of the sulfur and enveloping the heap in a mantle of flame and fusing the outer portion of the heap, and feeding successive portions of raw ore upon the surface of the heap and drawing off the molten product, as required. 20

In testimony whereof I affix my signature in presence of two witnesses.

JOHN W. MACDONALD.

Witnesses:

H. JOSEPH DOYLE,  
FRANK D. BLACKISTONE.